

## UNITED STATES PATENT OFFICE

2,126,742

## ALLOY

Anthony G. de Golyer, New York, N. Y.

No Drawing. Application April 17, 1936;  
Serial No. 75,020

3 Claims. (Cl. 148—32)

The present invention relates to a new and useful alloy and relates particularly to an alloy containing as essential components boron, zirconium, tungsten and cobalt, which has a high degree of hardness and other valuable properties.

This application is a continuation, in part, of my co-pending application, Serial No. 720,203, filed on April 12, 1934.

An object of the present invention is to provide an alloy especially adapted for use as metal cutting or forming tools, the cutting efficiency of which is several times greater than that of present known high speed steels and other alloys. A further object of this invention is to provide an alloy which is free from, or substantially free from carbon and which is readily amenable to thermal treatment, by means of which the hardness, tensile strength, cutting efficiency and other physical properties and characteristics may be accurately controlled over a comparatively wide range.

I have found through experiment that by alloying or otherwise intimately combining boron, zirconium, tungsten and cobalt within the range 25 boron from 0.50% to 5%, zirconium 1.50% to 20%, tungsten 10% to 40% and cobalt substantially the balance, that I obtain metallic compositions which possess in combination materially improved physical properties compared to those of heretofore known alloys or compositions intended for the cutting or working of metals.

Alloys of this invention may be used in the cast condition but approximate maximum values of hardness and certain other important physical properties can be developed only through thermal treatment, or through mechanical working and subsequent thermal treatment. Bodies of the alloys which have been subjected to such treatment are particularly valuable for use as tools, 40 dies and the like for the cutting or mechanical working of metals.

Numerous metallic compositions have heretofore been proposed as improvement on the generally known 18-4-1 type of tungsten-chromium-vanadium high speed tool steel, and while many of such compositions possess greater hardness than such steel, all of them have disadvantages which render them unsuitable for general application as metal cutting or forming tools. For 45 example, sintered or fused compositions containing principally carbides of tungsten, molybdenum or tantalum bonded with a relatively soft matrix metal have a high degree of hardness, but all of these are extremely brittle. Another disadvantage 50 is that such materials, when operated as metal

cutting tools at high speed, have a tendency to crater, i. e. to be worn away by contact with hot metal chips. Cast compositions such as the type comprising principally chromium, tungsten and cobalt, require the presence of at least 1.50% carbon to qualify as metal cutting tools, and, as is well known, such alloys are not only brittle, but are so sensitive to various operating conditions as to greatly restrict the scope of usefulness. One of the greatest disadvantages of virtually all of the heretofore suggested compositions is that none of them are responsive to thermal treatment for regulation of physical properties, and consequently physical properties and characteristics are governed entirely by the chemical composition of the 15 material.

My alloy may be used in the as-cast condition, or it may be forged and rolled or otherwise mechanically worked. I have found that both the cast and forged material are amenable to thermal treatment. For example, cast or forged bodies of this alloy may have a hardness of from 54 to 61 on the Rockwell C. scale and by subjecting the material to suitable thermal treatment, such as quenching from a temperature higher 20 than 1000° C., the hardness may be lowered to an approximate range of from 42 to 49 Rockwell C. In this condition the bodies may be ground, shaped or formed, if desired. The alloy may subsequently be submitted to a second thermal treatment, such as heating to a temperature of less 25 than 1000° C. for a period of from one or more hours, by which the hardness may be increased to from approximately 60 to 70 Rockwell C. In the latter condition the alloy is especially valuable 30 for the cutting or mechanical working of a large number of metals and alloys, as well as numerous non-metallic materials. An important property of the alloy is that virtually all of the maximum hardness, developed by thermal treatment, is retained when the alloy is subjected to elevated temperatures, e. g. such as are generated in the tip of a tool cutting metal at high speed. Another outstanding advantage is that 35 when the alloy of the present invention is used as a metal cutting tool, neither the tip nor any portion of the tool is burned or cratered by hot metal chips resulting from the cutting operation. Further hot chips do not adhere to the tool regardless of the speed at which it may be operated. In addition, the alloy is markedly 40 resistant to oxidation and corrosion at both normal and elevated temperatures. Although the alloy has a high degree of hardness, especially after 45

thermal treatment, it is remarkably resistant to failure from sudden or repeated shock.

The more important distinctive and valuable advantages are, apparently, due to the presence of appreciable amounts of boron in the composition, in conjunction with the other essential component elements within the percentages specified herein.

Although I usually prefer to have the alloy which is to be used as a metal cutting tool, for example composed principally of boron, zirconium, tungsten and cobalt, I have found that in many instances the tungsten may be supplanted in whole or in part by molybdenum or uranium, or both. The results of my investigations indicate that alloys composed principally of boron 0.50% to 5%, zirconium 1.50% to 20%, metal from the group molybdenum and uranium 10% to 40% and the balance cobalt, possess substantially the same valuable physical properties and characteristics as the above described composition containing only tungsten in combination with boron, zirconium and cobalt. Therefore, the alloy of my present invention comprises boron 0.50% to 5%, zirconium 1.50% to 20%, metal selected from the group tungsten, molybdenum and uranium 10% to 40% and the balance cobalt.

Specific examples of compositions within the scope of the present invention which I have found well adapted for use as metal cutting tools are the following: boron 1.40%, zirconium 7%, tungsten 12%, cobalt balance; boron 2.30%, zirconium 3%, tungsten 14.50%, cobalt balance; boron 1.20%, zirconium 9.50%, tungsten 19%, cobalt balance; boron 2.15%, zirconium 13%, molybdenum 12%, cobalt balance; boron 1.35%, zirconium 3%, tungsten 4%, molybdenum 10%, cobalt balance.

An objective of the present invention is to provide alloys having high hardness, advantageous metal cutting properties, etc., which are free or substantially free from carbon, and thus eliminate all of the serious disadvantages associated with carbon containing alloys or compositions intended for metal cutting tools. Although I prefer to have the alloys of this invention entirely free from carbon, in many instances I have found carbon present in the nature of an impurity incidental to manufacture. It is important to restrict the amount of carbon so present to a maximum of about 0.15%, as I have found that the presence of higher percentages of this element not only tend to embrittle the alloy, but

also to retard or inhibit the desired and necessary reactions during thermal treatment. Furthermore, the presence of appreciable amounts of carbon decreases the red hardness of the alloy, i. e. hardness at temperatures of approximately 550° C. and higher.

It will be understood that the alloys of the present invention may contain other elements as impurities incidental to manufacture. The amount of any one of such incidental impurities should be restricted to a maximum of 1% and in many instances to materially lower percentages.

My investigations indicate that the preferred structure of a body of the present alloy, particularly after thermal treatment, comprises at least two principal constituents: one, a relatively hard intermetallic compound of boron with one or more of the other essential components; and, second, a solid solution of two or more of the essential components which has a lower degree of hardness and functions as a matrix. In some instances the structure will contain a third constituent in the nature of an eutectoid. The ratio of the constituents in any particular body of the alloy may be accurately controlled and fixed over a wide range by means of thermal treatment, or mechanical working and subsequent thermal treatment.

By reason of the combined advantageous physical properties possessed by the alloy of the present invention, tools and other articles composed of this alloy may be operated efficiently and economically under conditions which are impossible or uneconomical with tools or articles composed of heretofore known alloys or metallic compositions.

It will be understood that the element vanadium may be added to the alloy of the present invention in an amount from approximately 0.25% to 2.50% but the inclusion of this element does not improve any of the physical properties.

I claim:

1. A precipitation hardened alloy consisting of boron 0.50% to 5%, zirconium 1.50% to 20%, metal from the group tungsten, molybdenum and uranium 10% to 40%, the balance cobalt.

2. A precipitation hardened alloy consisting of boron 0.50% to 5%, zirconium 1.50% to 20%, tungsten 10% to 40%, the balance cobalt.

3. A precipitation hardened alloy consisting of boron 0.50% to 5%, zirconium 1.50% to 20%, molybdenum 10% to 40%, the balance cobalt.

ANTHONY G. DE GOLYER.